

Nov. 6, 1951

P. MODIGLIANI  
METHOD OF FORMING A MULTILAYERED  
MAT OF INTERCROSSED FILAMENTS  
Filed March 16, 1946

2,574,221



INVENTOR.  
Piero Modigliani.

BY Virgil C. Kline  
ATTORNEY.

## UNITED STATES PATENT OFFICE

2,574,221

METHOD OF FORMING A MULTILAYERED  
MAT OF INTERCROSSED FILAMENTSPiero Modigliani, Manhasset, N. Y., assignor to  
Johns-Manville Corporation, New York, N. Y.,  
a corporation of New York

Application March 16, 1946, Serial No. 654,828

5 Claims. (Cl. 154—90)

1

The instant invention relates to an improved mat or sheet, and to the method of producing the same and, more particularly, to a filamentary glass article of this type and to the method of its production.

Heretofore filamentary sheets of glass and similar raw materials have been formed by various methods as shown, for example, in my prior Patent #2,081,060, issued May 18, 1937. As disclosed in said patent, glass fibers are drawn directly from a melting furnace or furnaces and accumulated on a rotating drum. The furnace and drum are relatively reciprocated so that the filaments of each of the layers accumulated on the drum are crossed suitably at acute angles to the filaments of adjacent layers. When the mat is built up to the desired thickness it is removed from the drum and stretched in a direction substantially perpendicular to the original lay of the filaments, whereby the mat is expanded or opened in a manner similar to that of a "lazy tongs," the angles between the fibers opening to increase the porosity and to reduce the density and thickness of the mat. The resultant mat has been employed both with and without the addition of an adhesive binder for many purposes.

The instant invention is particularly concerned with the provision of an improved mat which will have high strength and stretch-resistant characteristics in all directions. The invention also has for an object the provision of a mat with a glossy and more attractive surface than the mats heretofore obtained, the surface being subject to ornamentation. The mat may be used in many situations where the prior mats are not wholly successful, due to their surface characteristics, stretchability or other undesirable features eliminated by the instant construction.

Another object of the invention is the provision of a product including an expanded base mat or layer and a finish mat or layer on one surface of the base, the mats being integrated into a substantially unitary body.

A further object of the invention is the provision of a method of forming a product of a type attaining the foregoing objects.

A still further object of the invention is the provision of a method involving the production of an expanded mat and the accumulation on said mat of a filamentary surface layer in which the filaments lie approximately transversely to the fibers of the first mat.

A still further object of the invention is the provision of a method employing a filament-drawing apparatus such as a rotating drum of

2

substantially conventional type as a support for the first mat while the second mat is built up thereon.

My invention will be more fully understood and further objects and advantages thereof will become apparent when reference is made to the more detailed description of a preferred embodiment of the invention which is to follow and to the accompanying drawing in which:

10 Fig. 1 is a perspective view of a product of the instant invention;

Fig. 2 is a diagrammatic, elevational view of a portion of an apparatus employed in producing the product of Fig. 1;

15 Fig. 3 is a sectional view taken on the line 3—3 of Fig. 2;

Fig. 4 is a diagrammatic, perspective view of a mat of intercrossed glass filaments as employed in the instant invention and illustrating the condition of the mat before and after stretching operations;

Fig. 5 is a diagrammatic, end view of additional equipment employed in the production of the instant product; and,

20 Fig. 6 is a top plan view of the apparatus shown in Fig. 5.

Referring now to the drawings and particularly to Fig. 1, the product of the instant invention includes a base layer or mat 10 composed of 30 intercrossed, continuous or substantially continuous fine filaments 12. The mat is of preferably open, reticulated structure with the filaments crossing each other at approximately right angles to one another. Preferably fine glass filaments of a diameter range, say, between 6 and 18 microns make up the mats, although filaments of other sizes and/or other fusible materials may be employed. The filaments of mat 10 may be bound together by a suitable adhesive or binder as, for example, a water-soluble, thermo-setting resin, i. e., phenol-formaldehyde, urea formaldehyde or the like, or a binder such as gelatin. Water insoluble binders of any suitable type, such as polyvinyl alcohols, acryol, etc., or combinations of water-soluble and water insoluble binders may be employed. The binder is used in minor proportions, say, from 2-25% by weight of the mat, and is preferably disseminated substantially uniformly throughout the mat.

Overlying layer 10 is a second filamentary layer 14 also composed of substantially continuous filaments, suitably of the same kind employed in mat 10. The filaments 16 of this layer extend approximately transversely to the filaments of

mat 10 and are preferably in substantial parallelism. Filaments 16 are bound to each other and mats 10 and 14 are bound into a substantially integral product by an adhesive binder which may be of the same type as used in the formation of mat 10. However, the binders need not be the same in both mats, nor do the binders for either of the mats need to be selected from those specifically referred to, as any other adhesives having the properties desired for a particular service may be employed.

Filaments 12 and 16 are drawn from a fusible material, such as a glass melt, and in the manner fully explained below. Although the mats 10 and 14 have been referred to in some instances as layers, it will be understood that each is made up of a plurality of laps or laminations of the glass filaments to produce a body of appreciable thickness. Also, although the filaments of mat 14 preferably all lie in approximate parallelism, this is not critical and they may also intercross to a substantial extent, as long as they extend approximately transversely to the lay of the fibers in mat 10.

Surface layer or mat 14, particularly when the fibers are in substantial parallelism as in the preferred construction provides a glossy, light-reflective surface which adapts the product for use as a decorative medium and for other purposes for which the expanded mat 10 alone is not suitable. The glossy, light-reflective surface of the product may be printed or otherwise decorated and also mat 14 may be colored as desired.

Referring now particularly to Figs. 2-6, the method of forming the product described above will be explained in detail. Mat 10 is preferably fabricated by following substantially the conventional practice as described, for example, in my said Patent #2,081,060. In Figs. 2 and 3, there is diagrammatically shown a filament accumulating or drawing drum 18 of the type employed in the patented method. The fiber integrally connected to glass issuing through the spinning orifices of a glass furnace 20 of any suitable type is brought into contact with the drum and continuously drawn directly from the glass furnace by rotation of the drum in the direction indicated by the arrow. Furnace 20 is reciprocated relatively to the drum, as indicated by the double-headed arrow in Fig. 3, to lay the glass filaments onto the drum in a plurality of layers of continuous spirals, with the filaments of each layer crossing the filaments of adjacent layers. When the mat is built up to the desired thickness on drum 18, it is removed, suitably by slitting it axially of the drum, and is transferred to a conveyor or the like 22 which feeds it to a stretching device, indicated generally at 24. The stretching device may be of the type shown, for example, in my said Patent #2,081,060, but preferably an apparatus of the type described and claimed in the co-pending application of Robert E. Slack et al., S. N. 606,247, filed July 20, 1945, now Patent No. 2,486,217, is employed to secure a superior product.

Referring particularly to Fig. 4, the effect of the stretching operation is diagrammatically illustrated. The mat, as received from the drum, conventionally referred to at this stage as a "condensed mat," is indicated by the reference character 26 and, after the stretching operation, is indicated by the reference character 28. As shown, the angular relationship between the fibers is altered as the mat is drawn or stretched, to produce a thinner, more open, reticulated structure.

The mat, after leaving the stretching rolls, is treated with an adhesive as it passes under an adhesive applicator 30. A binder or adhesive of any of the types previously referred to is sprayed onto the mat by the applicator, the adhesive penetrating into the thin, open mat. The treated mat then travels through an oven or other suitable setting chamber 32 in which the adhesive is set and hardened. A section 33, indicated by the dot-dash lines 34 of Fig. 4, is then cut from the mat, the section being of a length  $a$  equal to the circumference of a fiber-drawing or accumulator drum which may be drum 18 employed for the original fiber-drawing operation or which may be a separate, but preferably similar drum as shown at 36 in Figs. 5 and 6. Section 33 is wrapped onto the drum with its longitudinal dimension  $a$  extending circumferentially of the drum and secured by connecting the end edges with strips of adhesive tape or the like 38. Drum 36 is then rotated and filaments 16 drawn from a glass furnace (not shown) which may be furnace 20 or one similar in all respects to furnace 20, and the drawn filaments wrapped on the drum to overlie mat 10 and form a surfacing layer or mat thereon. The fiber drawing is continued to wind a plurality of laps or layers of the filaments to build up a mat of the desired thickness. Suitably the reciprocation of the furnace or of the drum, as the case may be, is relatively slow to lay the filaments of the second laps or layers in substantial parallelism, with the filaments extending approximately at right angles to the axis of the drum. However, the rate of reciprocation may be such as to lay the filaments in layers at acute angles to adjacent layers, similarly as in the formation of the original mat on the drum 18 but the more parallel accumulation of the filaments is preferred, as previously pointed out.

An adhesive or binder such as a water-soluble resin or gelatin, or a combination of water-soluble binders and water-insoluble binders, as referred to above, is sprayed onto the filaments or onto the mat of filaments as the filaments are accumulated. For this purpose a spray device 40 is located adjacent the point of wrapping of the filaments on the drum. The spray device may be of any suitable type comprising, for example, a pipe extending longitudinally of the drum, the pipe being connected to any suitable binder supply. The pipe is provided with a plurality of nozzles directed toward the drum. The ports or nozzles are relatively small to spray the binder against the drum in finely-divided or atomized form.

Drying means are employed to set the binder as the mat 14 is accumulated on the drum. Such drying means, indicated generally at 42, may be of any suitable or conventional type such as a battery of infra-red ray lamps, gas burners or the like. The drying means serves to set up the adhesive so that the combined product, when the mat 14 is built up to the desired thickness, may be directly removed from the drum. After removal, the mat is divided into segments of the selected size for the particular use for which the product is intended.

If desired a coloring material such as any of the known coloring compositions may be sprayed onto the mat 14 during its formation to insure uniform depth of color of the surfacing layer. The coloring material may be included with the binder or may be supplied by a separate spray device, indicated at 44.

The method described above provides a simple, effective and economical way of producing the product as shown in Fig. 1. The product may be varied in a number of particulars without the necessity of making major adjustments in the method or apparatus by which it is produced. The mat 10 may be expanded to any extent desired, within the limits permitted by the character of the material, during the stretching operation to provide a base mat of greater or lesser porosity, thickness and strength by merely properly adjusting the speed of the drawing mechanism. The surface mat may consist of substantially parallel fibers or of intercrossed fibers, by proper adjustment of the rate of traverse of the furnace relative to the drum during the accumulation of the mat on the base mat 10. Various colors may be employed in any suitable or desired arrangement.

Having thus described my invention in rather full detail, it will be understood that these details need not be strictly adhered to but that various changes and modifications may suggest themselves to one skilled in the art, all falling within the scope of the invention as defined by the subjoined claims.

What I claim is:

1. The method comprising forming a multi-layer mat of intercrossed filaments, stretching said mat, accumulating a second filamentary mat on said first mat with the filaments of said second mat extending generally in the direction of stretch of said first mat, and adhesively securing the second mat to the first mat.

2. The method comprising forming a multi-layer mat of intercrossed filaments, stretching said mat, applying an adhesive to said stretched mat, accumulating a second filamentary mat on said first mat with the filaments of the second mat extending generally in the direction of stretch of the first mat, and applying an adhesive to said filaments of said second mat as they are accumulated.

3. The method comprising forming a multi-layer mat of intercrossed filaments, stretching said mat, applying an adhesive to said mat, placing said mat on a filament accumulating device, simultaneously drawing filaments from

6

a raw material supply and collecting them on said mat, and applying adhesive to said filaments as they are drawn.

4. The method comprising forming a multi-layer mat of intercrossed filaments, stretching said mat, placing said mat on a rotatable fiber drawing drum, accumulating a second multi-layer mat of newly drawn fibers directly on said first mat on said drum, applying adhesive to said filaments as they are drawn, and setting said adhesive while said mat and filaments are on said drum simultaneously with the fiber drawing operation.

5. The method comprising forming a filamentary mat having a plurality of coextensive layers with the filaments of each layer in substantial parallelism and in intercrossing relationship with the filaments of adjacent layers, stretching said mat to increase the angular relationship between the filaments of the layers and to produce a more open, reticulated structure, accumulating a second filamentary mat on said first mat with the filaments of said second mat extending generally longitudinally of the first mat and crossing the filaments thereof, and adhering the filaments of said mat together, and said second mat to said first mat.

PIERO MODIGLIANI.

#### REFERENCES CITED

The following references are of record in the file of this patent:

#### UNITED STATES PATENTS

| Number    | Name           | Date           |
|-----------|----------------|----------------|
| 1,771,216 | Gossler        | July 22, 1930  |
| 2,015,006 | Ekisler        | Sept. 17, 1935 |
| 2,081,060 | Modigliani     | May 18, 1937   |
| 2,117,371 | Slayter        | May 17, 1938   |
| 2,131,024 | Cordts         | Sept. 27, 1938 |
| 2,306,347 | Slayter        | Dec. 22, 1942  |
| 2,315,851 | Goldman        | Apr. 6, 1943   |
| 2,397,936 | Glidden et al. | Apr. 9, 1946   |
| 2,399,258 | Taylor         | Apr. 30, 1946  |

#### FOREIGN PATENTS

| Number  | Country       | Date          |
|---------|---------------|---------------|
| 323,790 | Great Britain | Jan. 16, 1930 |